

## UNITED STATES PATENT OFFICE

GEORGE HOLLAND ELLIS, OF SPONDON, NEAR DERBY, ENGLAND, ASSIGNOR TO  
CELANESE CORPORATION OF AMERICA, A CORPORATION OF DELAWARE

## TREATMENT OF MATERIALS CONTAINING NATURAL SILK

No Drawing. Application filed June 24, 1929, Serial No. 373,490, and in Great Britain July 9, 1928.

This invention relates to the treatment of fabrics or other goods or materials made of or containing natural silk with alkaline reagents.

It is well-known that treatment of materials containing natural silk with caustic alkali results in degradation of the silk. In degumming materials comprising natural silk it has been the practice to temper the action of caustic alkali by addition of other reagents such as sulphonated oil or to use instead of caustic alkali, alkaline reagents having a milder action, for example borax or sodium silicate.

I have now made the discovery that natural silk goods may be protected against the action of alkaline reagents by the simultaneous presence of cellulose esters. Provided that the latter be present in more than an insignificant percentage, the action of the alkali is almost wholly confined to the cellulose ester component, the natural silk remaining substantially unaffected. This discovery is very surprising since it would be expected that the natural silk already degummed or degummed by reason of the alkaline reagent would be acted upon by the alkaline reagent to produce a degradation in addition to saponification or hydrolysis of the cellulose ester. This discovery may be most usefully applied in the treatment of mixed materials containing both natural silk and cellulose acetate or other cellulose esters. By treating such a mixed material with a suitable alkaline reagent saponification of the cellulose ester results with or without degumming of the natural silk but without degradation.

In the past in degumming the natural silk of materials comprising both cellulose esters and natural silk care has been taken to avoid alkalinity sufficient to produce either degradation of the natural silk constituent or saponification or hydrolysis of the cellulose ester.

I have found moreover that the above property may be utilized to produce various colour effects upon mixed materials containing both cellulose esters and natural silk. For example, the material containing natural silk and superficially or partially saponi-

fied cellulose ester may be treated with dyestuffs, for instance some acid and direct cotton dyestuffs, having an affinity for the natural silk and for cellulose materials to produce shades substantially even on the cellulose ester and silk components.

Moreover I have found that the superficially or partially saponified or hydrolyzed cellulose esters retain their affinity for the insoluble colours especially devised for application to cellulose esters and usually applied in solubilized or dispersed form, e. g. the "S. R. A. colours". By applying such dyestuffs for dyeing the cellulose ester constituent of the mixed materials, differential colouration is obtainable since the natural silk is not in general dyed by these dyestuffs. Furthermore the materials treated according to the present invention may be dyed both with the "S. R. A." type of colour and with the direct cotton type of colour so as to obtain a single shade on the natural silk due to the direct cotton colour and a compound shade on the cellulose ester component due to both types of colour. Again if desired the mixed materials treated according to the present invention may be coloured with acid dyestuffs which resist or only slightly stain cellulosic materials and this type of dye may be applied in conjunction with any of the other types previously mentioned. The coloured effects may be obtained on the goods by any suitable methods of colouration, for example dyeing, printing, stenciling and the like.

In carrying out the treatment with alkaline reagents according to the present invention any suitable alkalies capable of producing a superficial or partial saponification or hydrolysis of the cellulose ester may be employed, and furthermore salts or other electrolytes may be added thereto as has been proposed in prior saponification processes. The treatment with an alkaline reagent may conveniently and economically be carried out in conjunction with the degumming of the natural silk by simple addition of the sufficient quantities of alkali to the customary soap or soluble or sulphonated oil solution. Furthermore if desired dye-

stuffs may be incorporated in such a solution provided they are compatible therewith, for example the insoluble dyestuffs generally applied to cellulose esters in solubilized or dispersed form.

I have found that the best results in the saponification or hydrolysis are obtained if the liquor, bath volume is adjusted so as to have a minimum ratio of 40:1 on the weight of the goods.

By effecting the treatment at a sufficiently high temperature, e. g. above 90° C., the lustre of the cellulose ester portion may be modified.

The following examples illustrate the invention, but are not to be considered as limiting it:

#### Example 1

A woven crepe fabric consisting of equal 20 weights of cellulose acetate and natural silk in the gum is suspended by means of loops in a 40:1 bath containing 5 grams per litre of soap and a quantity of caustic soda equal to 10% of the weight of cellulose acetate present. The bath is then raised to 95-100° C. and the goods treated for 3 hours, by which time the cellulose acetate is saponified approximately 10%, lustre being simultaneously modified. The natural silk is simultaneously fully degummed, loss in weight being normal, and handle and tensile strength fully equal to samples degummed by methods familiar in the art.

The cellulose acetate portion may now be 35 dyed with the insoluble dyestuffs having selective affinity for that fibre, and the natural silk with acid dyestuffs having little or no affinity for cellulose acetate or regenerated cellulosic fibres. Thus a blue may be obtained 40 on the cellulose acetate by means of dimethyldiamino-anthrarufin, and an orange on the natural silk with Kiton Fast Orange G. (Colour Index No. 27).

#### Example 2

A woven crepe fabric consisting of 1 part of degummed natural silk as weft and 2 parts of cellulose acetate as warp is treated at 80° C. in a 5 gram per litre soap solution containing 5% caustic soda on the weight of cellulose acetate (volume 200:1). A further 2½% caustic soda is added after 1 hour, and a similar amount again after another ½ hour making 10% in all. Treatment is continued for ½-1 hour longer, after which the fabric is lifted, rinsed and dried or otherwise treated as requisite. The cellulose acetate portion has now been saponified approximately 10% 55 and exhibits the modified dyeing and other properties of superficially or partially saponified cellulose acetate, whilst the natural silk retains its characteristic properties.

While the invention has been described 60 above more particularly with reference to the

treatment of materials consisting of natural silk and cellulose acetate it may be applied to materials consisting of natural silk and other cellulose esters, for instance cellulose formate, cellulose propionate, cellulose butyrate or the products obtained by treatment of alkali cellulose with esterifying agents, e. g. the product obtained with p-toluene sulpho-chloride and known as "immunized cotton" and to materials containing other constituents in addition to natural silk and cellulose esters, for example cotton or other natural cellulose material, cellulose ethers, or the cellulosic type of artificial silk, i. e. viscose, cuprammonium or nitrocellulose artificial silk. Such other constituents may be dyed or otherwise coloured with any of the usual dyestuffs therefor to produce further effects.

What I claim and desire to secure by Letters Patent is:—

1. In the treatment of materials comprising natural silk with alkaline liquors, the step of protecting the natural silk against the action of the alkaline reagents by effecting the treatment in the presence of cellulose ester material.

2. In the treatment of materials comprising natural silk with alkaline liquors, the step of protecting the natural silk against the action of the alkaline reagents by treating it in the form of a mixed material with a cellulose ester.

3. In the treatment of materials comprising natural silk with alkaline liquors, the step of protecting the natural silk against the action of the alkaline reagents by treating it in the form of a mixed material with a cellulose ester, the reagents being sufficiently alkaline to produce partial saponification of the cellulose ester.

4. In the degumming of materials comprising natural silk with alkaline liquors, the step of protecting the natural silk against the action of the alkaline reagents by treating it in the form of a mixed material with a cellulose ester.

5. In the treatment of materials comprising natural silk with alkaline liquors, the step of protecting the natural silk against the action of the alkaline reagents by effecting the treatment in the presence of cellulose acetate material.

6. In the treatment of materials comprising natural silk with alkaline liquors, the step of protecting the natural silk against the action of the alkaline reagents by treating it in the form of a mixed material with cellulose acetate.

7. In the treatment of materials comprising natural silk with alkaline liquors, the step of protecting the natural silk against the action of the alkaline reagents by treating it in the form of a mixed material with cellulose acetate, the reagents being suffi-

sufficiently alkaline to produce partial saponification of the cellulose acetate.

8. In the degumming of materials comprising natural silk with alkaline liquors, the step of protecting the natural silk against the action of the alkaline reagents by treating it in the form of a mixed material with cellulose acetate.

9. In the treatment of materials comprising natural silk with alkaline liquors, the step of protecting the natural silk against the action of the alkaline reagents by treating it in the form of a mixed material with a cellulose ester and subsequently colouring the material with a dyestuff having an affinity for at least one of the constituents of the mixed material.

10. In the treatment of materials comprising natural silk with alkaline liquors, the step of protecting the natural silk against the action of the alkaline reagents by treating it in the form of a mixed material with cellulose acetate and subsequently colouring the material with a dyestuff having an affinity for at least one of the constituents of the mixed material.

11. In the treatment of materials comprising natural silk with alkaline liquors, the step of protecting the natural silk against the action of the alkaline reagents by treating it in the form of a mixed material with a cellulose ester, the reagents being sufficiently alkaline to produce partial saponification of the cellulose ester and subsequently colouring the material with a dyestuff having an affinity for both of the constituents of the mixed material.

12. In the treatment of materials comprising natural silk with alkaline liquors, the step of protecting the natural silk against the action of the alkaline reagents by treating it in the form of a mixed material with cellulose acetate, the reagents being sufficiently alkaline to produce partial saponification of the cellulose acetate and subsequently colouring the material with a dyestuff having an affinity for both of the constituents of the mixed material.

In testimony whereof I have hereunto subscribed my name.

50 GEORGE HOLLAND ELLIS.